

## UNITED STATES PATENT OFFICE

2,495,668

## ELECTRODEPOSITION OF COPPER

Karl S. Willson and David G. Ellis, Cleveland,  
Ohio, assignors to The Harshaw Chemical  
Company, Elyria, Ohio, a corporation of Ohio

No Drawing. Application December 21, 1946,  
Serial No. 717,800

5 Claims. (Cl. 204—52)

1

This invention relates to electrodeposition of copper and more particularly to improved processes and solutions for electrodeposition of bright copper.

We have now discovered that excellent bright copper deposits can be made by the inclusion in the copper cyanide plating solution of a suitable quantity of an organic compound of the class consisting of:

B-mercaptop ethanol ( $\text{HOCH}_2\text{CH}_2\text{SH}$ )  
Di thio diglycol ( $\text{HOCH}_2\text{CH}_2\text{SSCH}_2\text{CH}_2\text{OH}$ )  
B,B' dihydroxyethyl sulfide  
( $\text{HOCH}_2\text{CH}_2\text{SCH}_2\text{CH}_2\text{OH}$ )  
Thioglycollic acid ( $\text{HOOCCH}_2\text{SH}$ )

That is, when such a deposit is made, it can be built up to substantial thickness, three ten-thousandths of an inch and more, and still exhibit greatly improved lustre as compared with the usual cyanide copper bath. Agitation of the solution results in improvement in lustre and makes possible the use of much higher current density, e. g. increase from 10 a. s. f. to 60 a. s. f. Interruption of the current at intervals, e. g. 1 minute on, 10 seconds off, reversal of the current every few seconds or use of alternating current superimposed on the direct current, all tend to produce improved lustre and more uniform deposits.

The compound to be suitable should have adequate solubility in the copper cyanide bath to make possible the maintenance in solution of a sufficient quantity of the addition agent to achieve the desired result. The concentration of addition agent required for best results varies among the above indicated addition agents. In the case of B-mercaptop ethanol the concentration should not be less than 0.05 gram per liter nor more than 10 grams per liter, a preferred range being from about 1 to 4 grams per liter. In the case of dithio diglycol, the concentration should not be less than 0.04 gram per liter nor more than 1.8 grams per liter, the optimum being from about 0.6 to 1.0 gram per liter. In the case of thioglycollic acid, the concentrations may be rather low, not less than about 0.007 gram per liter but may also be as high as 35 grams per liter, a preferred range being from 0.25 to 15 grams per liter. In the case of B,B' dihydroxyethyl sulfide the concentration may run from 1 gram per liter to as high as 240 grams per liter, a preferred range being from 4 to 70 grams per liter.

An aqueous alkaline plating bath may be employed containing 4 to 20 ounces (30 to 150 grams per liter) of CuCN per gallon and the requisite

amount of NaCN. The preferred pH range is 9.5 to 11.5 but good results may be had from 8.5 to 12.5. Free cyanide content may be from 0 to 11.5 grams per liter or more, the preferred range being 2 to 12 grams per liter. In general, increase of free cyanide is desirable with increasing CuCN content. The temperature is preferably maintained between 130° F. and 150° F. although good results can be had between 120° F. and 160° F.

10 Current is passed through the above indicated solutions from a copper anode to a cathode at a cathode current density of from a very low value up to 60 amperes per square foot.

Preferred solutions and plating conditions 15 would be, for example:

## Example I

|                         |                 |     |
|-------------------------|-----------------|-----|
| CuCN                    | grams per liter | 30  |
| Free cyanide            | do              | 12  |
| 20 B-mercaptop ethanol  | do              | 4   |
| Water                   | Remainder       |     |
| pH                      |                 | 8.5 |
| CD (continuous current) | a. s. f.        | 30  |
| Temperature             | °F              | 140 |

25

## Example II

|                         |                 |      |
|-------------------------|-----------------|------|
| CuCN                    | grams per liter | 120  |
| Free cyanide            | do              | 5    |
| 30 Dithiodiglycol       | do              | 0.6  |
| Water                   | Remainder       |      |
| pH                      |                 | 12.5 |
| CD (continuous current) | a. s. f.        | 20   |
| Temperature             | °F              | 140  |

35

## Example III

|                                                      |                 |      |
|------------------------------------------------------|-----------------|------|
| CuCN                                                 | grams per liter | 120  |
| Free cyanide                                         | do              | 12   |
| 40 B,B' dihydroxyethyl sulfide                       | do              | 70   |
| Water                                                | Remainder       |      |
| pH                                                   |                 | 12.5 |
| C. D. (interrupted current, 30 sec. on; 10 sec. off) | a. s. f.        | 15   |

45

This bath gave brighter deposits with interrupted current than with continuous current.

## Example IV

|                         |                 |      |
|-------------------------|-----------------|------|
| CuCN                    | grams per liter | 30   |
| 50 Free cyanide         | do              | 2    |
| Thioglycollic acid      | do              | 20   |
| Water                   | Remainder       |      |
| pH                      |                 | 10.0 |
| CD (continuous current) | a. s. f.        | 20   |
| Temperature             | °F              | 140  |

55

Having thus described our invention, what we claim is:

1. An aqueous, alkaline electroplating bath which comprises an aqueous medium to which has been added a metal ion yielding material essentially consisting of copper cyanide in concentration from 30 to 150 grams per liter, a sufficient amount of sodium cyanide to produce from 2 to 12 grams per liter of free cyanide in the solution and an amount of a brightening addition agent of the class consisting of B-mercapto ethanol, dithiodiglycol, B,B' dihydroxyethyl sulfide and thioglycollic acid sufficient to permit a brilliant cathodic deposit of copper upon the passage of an electric current from a copper anode to a cathode through the bath, the concentration of said brightening addition agent being from 0.05 gram per liter to 10 grams per liter in the case of B-mercapto ethanol, from 0.04 gram per liter to 1.8 grams per liter in the case of dithiodiglycol, from 0.007 gram per liter to 35 grams per liter in the case of thioglycollic acid, and from 1 gram per liter to 240 grams per liter in the case of B,B' dihydroxyethyl sulfide.

2. A method which comprises electrodepositing copper from an aqueous, alkaline copper cyanide solution containing from 30 to 150 grams per liter of copper cyanide and from 2 to 12 grams per liter of free cyanide, there being added to such solution as a brightening agent a substance of the class consisting of B-mercapto ethanol, dithiodiglycol, B,B' dihydroxyethyl sulfide and thioglycollic acid, the concentration of said brightening addition agent being from 0.05 gram per liter to 10 grams per liter in the case of B-mercapto ethanol, from 0.04 gram per liter to 1.8 grams per liter in the case of dithiodiglycol, from 0.007 gram per liter to 35 grams per liter in the case of thioglycollic acid, and from 1 gram per liter to 240 grams per liter in the case of B,B' dihydroxyethyl sulfide.

3. An aqueous, alkaline electroplating bath which comprises an aqueous medium to which has been added a metal ion yielding material essentially consisting of copper cyanide in con-

centration from 30 to 150 grams per liter, a sufficient amount of sodium cyanide to produce from 2 to 12 grams per liter of free cyanide in the solution and containing as an organic brightening addition agent B-mercapto ethanol in concentration from 0.05 to 10 grams per liter.

4. An aqueous, alkaline electroplating bath which comprises an aqueous medium to which has been added a metal ion yielding material essentially consisting of copper cyanide in concentration from 30 to 150 grams per liter, a sufficient amount of sodium cyanide to produce from 2 to 12 grams per liter of free cyanide in the solution and containing as an organic brightening addition agent B,B' dihydroxyethyl sulfide in concentration from 1 to 240 grams per liter.

5. An aqueous, alkaline electroplating bath which comprises an aqueous medium to which has been added a metal ion yielding material essentially consisting of copper cyanide in concentration from 30 to 150 grams per liter, a sufficient amount of sodium cyanide to produce from 2 to 12 grams per liter of free cyanide in the solution and containing as an organic brightening addition agent dithiodiglycol in concentration from 0.04 to 1.8 grams per liter.

KARL S. WILLSON.  
DAVID G. ELLIS.

#### REFERENCES CITED

The following references are of record in the file of this patent:

#### UNITED STATES PATENTS

| 35 | Number    | Name                  | Date          |
|----|-----------|-----------------------|---------------|
|    | 2,147,415 | Tucker -----          | Feb. 14, 1939 |
|    | 2,195,409 | Flett -----           | July 29, 1940 |
|    | 2,402,640 | Lazier et al. -----   | June 25, 1946 |
|    | 2,410,844 | Signaigo et al. ----- | Nov. 12, 1946 |
| 40 | 2,424,887 | Henricks -----        | Apr. 2, 1947  |

#### OTHER REFERENCES

The Metal Industry, March 1943, pages 134-137, and Apr. 1, 1943, page 206.